

Patented July 17, 1928.

1,677,389

# UNITED STATES PATENT OFFICE.

RAYMOND T. HOWES, OF WILMINGTON, CALIFORNIA, ASSIGNOR TO PAN AMERICAN PETROLEUM COMPANY, OF LOS ANGELES, CALIFORNIA, A CORPORATION OF CALIFORNIA.

## CYLINDER-OIL COMPOSITION AND METHOD OF PREPARING SAME.

No Drawing.

Application filed January 5, 1927. Serial No. 159,844.

This invention relates to oils for use primarily in hydrostatic sight feed lubricators, in which oil, emerging in drops or globules from the jet or nozzle of such devices, passes 5 through liquid in a section of tubing of transparent material, so that the rate of supply of the lubricating oil may be observed.

Because of the comparative high specific 10 gravity and high surface tension of oils having an asphaltic or naphthenic base as indicated in California crude petroleum stock, it is very difficult to obtain a cylinder oil which will feed satisfactorily in a sight feed lubricator. It is found that cylinder 15 stock made from California crude petroleum oil or oil having an asphaltic or naphthenic base, exhibit a surface tension inherently greater than stock made from the eastern 20 oils or crudes of lighter specific gravity and surface tension, and because of these characteristics, globules of such oil of the heavy California crudes resist for a longer period 25 of separation from the jet or nozzle, with the result that during the attenuation of the oil film prior to severance thereof from the jet, the globule attains a comparatively large size, which ascends sluggishly in the buoyant 30 fluid in the section of glass tubing. Large 35 globules or drops are objectionable, because in the first place the time required for their formation, owing to tenacious surface tension, curtails and interferes with efficient lubrication, and in the second place, interferes with proper and ready observation.

The object of this invention, therefore, is to provide an oil for lubricating purposes, and especially adapted for sight feed lubricators in which the surface tension of the oil 40 is reduced to that degree that the oil globules may be formed quickly of satisfactory size and speedily separated from the jet, and rise in their fluid surroundings without retardation due to rubbing friction which is the 45 objectionable characteristic of oversized and deformed globules.

Globules of oil made from California crude, which has been treated to reduce the 50 normal surface tension thereof are very much smaller and have a regular sphericity as compared to the vacillating sphericity of bulky and oversized globules, the flatness and deformity of which indicate a lower surface tension. For this reason, a closer and

better observation of the lubricator may be 55 had than with globules having a sluggish buoyancy.

I have discovered that by mixing with a cylinder oil made from California crude stock certain sulphonated oils, the surface 60 tension of the cylinder oil is reduced considerably and that such an oil composition will enable smaller globules to emerge from the jet or nozzle of the lubricator, with increased acceleration so soon as the surface 65 tension of same is sufficient to overcome their cohesion.

The sulphonated oil which I prefer to use is the product resulting from the interaction 70 of ammonia and sulfonated corn or cotton seed oil. The product bears the trade name "Turkey red oil," which is readily soluble in cylinder oil and which, I have found, reduces the surface tension for the purposes mentioned.

In practice, the proportion which the "Turkey red oil" sustains to the cylinder 75 stock is, about 2.5%, and the mixture is prepared at any convenient temperature, below the decomposition point of the sulphonated 80 oil, through agitation.

I have found the "Turkey red oil" to be very effective in reducing the surface tension of cylinder oil made from California crudes, but there are other compounds and 85 substances which, when added to the cylinder oil stock, will produce a like effect upon the oil in causing a small globule to be formed at, and to part from the jet or nozzle so soon as the buoyancy thereof overcomes the co- 90 hesiveness of the globules. Such compounds for reducing the surface tension of cylinder oils includes the sulfonated petroleum acids from petroleum, which petroleum acids are the sludges produced by the treatment of pe- 95 troleum oils with sulfuric acid. These and other compounds and groups of substances that operate to reduce the surface tension of the cylinder oil stock, either directly or indirectly are included in this disclosure. 100 Such substances or compounds which indirectly operate to produce or bring about the formation of smaller globules with low surface tension, are those which, when commingled with water are partly or wholly dissolved and provide an environment which effects reduction of surface tension of globule formed at the jet or nozzle. A compound of

this kind may be a soap which will render the fluid in the glass of the lubricator soapy and may be mixed directly with the cylinder oil, or the globules of the cylinder oil, unchanged by added compounds, may enter and form in a soapy fluid, in which event a like effect of the globule will be had. While the latter expedient may be resorted to with good results, I have found that compounding the cylinder oil as disclosed, with "Turkey red oil", works to better advantage in producing globules, the cohesiveness of which is to be reduced to the point where small uniform globules will readily separate from the jet with continuous regularity.

As a specific example of a cylinder oil compound suitable for hydrostatic sight-feed lubricators, I may employ any high viscosity lubricating oil made from a California crude oil such for example, as a cylinder oil made from the crude oil obtained from Elk Hills, Kern County, California, and one which has a viscosity of approximately 154 seconds Saybolt at 210 degrees F. Preferably, about 2½ per cent of "Turkey red" oil is added to the cylinder oil and the mass agitated until a uniform mixture is obtained. The mixing may be facilitated by heating the mixture to a temperature ranging from 100 to 180 degrees F. or a little higher if desired. The time required for making this mix depends upon the size of the batch, the

temperature employed and rate of agitation which may range from 15 minutes to 1 hour or a little longer, if very large batches are to be mixed. The following shows the physical test on a sample of cylinder oil made from an asphalt base crude petroleum oil obtained from Elk Hills, Kern County, California, before and after the addition of 2½ per cent of "Turkey red" oil: gravity, 18.2° Baumé; flash, 515° Fahr.; fire test, 595° Fahr.; viscosity at 210° F. Saybolt 154 seconds.

After being commingled with 2½ per cent of "Turkey red" oil: gravity, 18.1° Baumé; flash 515° F.; fire test, 595° F., viscosity at 210° F. Saybolt 153 seconds.

It will be noticed that there is substantially no difference in the above physical test before and after the cylinder oil is compounded with the "Turkey red" oil. However, there is a decrease in the surface tension which the applicant has no direct means of measuring.

What I claim, is:

A process of reducing the surface tension of cylinder oil made from California crude petroleum stock, for use in hydrostatic sight-feed lubricators, which consists in mixing with the cylinder oil approximately two and one half per centum of Turkey red oil.

In testimony whereof I have set my hand.  
RAYMOND T. HOWES.